

(No Model.)

G. D. BARTLETT.  
TUMBLING STAR.

No. 591,225.

Patented Oct. 5, 1897.



Witnesses:

G. L. Cartman.

M. F. Boyle.

Inventor  
George D. Bartlett  
By James Drew Stetson  
Attorney.

# UNITED STATES PATENT OFFICE.

GEORGE D. BARTLETT, OF PLYMOUTH, MASSACHUSETTS.

## TUMBLING-STAR.

SPECIFICATION forming part of Letters Patent No. 591,225, dated October 5, 1897.

Application filed January 11, 1896. Serial No. 575,073. (No model.)

To all whom it may concern:

Be it known that I, GEORGE D. BARTLETT, of Plymouth, Plymouth county, in the State of Massachusetts, have invented a certain new and useful Improvement in Tumbling-Stars, of which the following is a specification.

The invention relates to means for cleaning small castings by tumbling in a revolving case or box to remove the adhering material composed of molding earth more or less baked by the intense heat to which it has been subjected when the iron was in a melted state. It is common to tumble the castings with a quantity of loose pieces technically known as "tumbling-stars," and the castings are more rapidly and thoroughly cleaned by reason of the action of these added pieces on the surfaces. It is important that the tumbling-stars shall be hard and of such form that they will act in all the reentering angles of the castings. I make the tumbling-stars of sheet metal, high steel, about No. 16, Birmingham gage. I cut the sheets into small square pieces and stamp them into dishing form, crimp, and harden them.

The accompanying drawings form a part of this specification and represent what I consider the best means of carrying out the invention.

Figure 1 is a view of the full side of one of my tumbling-stars. Fig. 2 is a section on the line 2 2 in Fig. 1. Fig. 3 is a view of the hollow side, and Fig. 4 is a section on the line 4 4 in Fig. 1. Fig. 5 is a section corresponding to Fig. 2, but showing the same tumbling-star after it has been much worn. Fig. 6 is a view corresponding to Fig. 3, showing the star in the same worn condition. Fig. 7 shows the blank before it is treated in the dies. The dotted lines thereon indicate the skewed position of the indentations produced by the dies in the act of stamping.

Similar letters of reference indicate corresponding parts in all the figures where they appear.

I roll plates of high steel down to a thickness of about a sixteenth of an inch and, having them properly heated, cut them into square blanks and stamp them each into a star form, as indicated in the figures.

A is the body of the metal, and A' the points which were the corners of the original square blanks.

A<sup>2</sup> are recesses produced by crimping, deflecting, or dishing the metal strongly midway between each point and the next. The form may be induced by compressing the sheet metal in a heated state between two dies of the required form. The blanks are set a little askew relatively to the dies, and the effect is to bend the metal slightly hookwise at the several points, so as to give increased sharpness, as indicated by A<sup>3</sup>. This form gives superior action to the several points while the stars are new. I will designate by B the cross-marks produced by the action of the dies in the hollow sides.

My sheet-metal tumbling-stars thus produced, dished and made angular, may be hardened at the same heat, as the shaping is effected by simply dropping them from the dies into cold water. They may, if preferred, be separately heated and plunged into water which has been doctored with salt or other material to get the highest degree of hardness. A liberal quantity of these stars are placed in the tumbling-barrel with the castings to be cleaned, and as the work proceeds their thin edges are presented irregularly to all parts of the castings the same as the ordinary tumbling-stars, but the fact that they are of sheet-steel, treated as described, gives them superior hardness, so that a given quantity of my stars will serve for a long period without appreciable wear. The form gives the quality that they continue to present effective working edges after they have been much worn. The sheet-metal stars, unlike the castings ordinarily used for this purpose, present the same thickness at their edges after they have been worn away to a quarter or any other fraction of their original sizes.

By making my tumbling-stars from sheet metal of the form shown I am enabled to use all the material and to cut it to the required angular shape with ordinary tools and labor.

My improved tumbling-stars may be used in all respects in the ordinary manner. I can use the ordinary means, as screening or winnowing, to separate my stars from the cast-

ings and from the more or less pulverized scale which the tumbling operation has removed.

Instead of using high steel I can use soft steel or simply iron as the material for my sheet metal, and after the pieces have been cut and pressed, which may with such material be done cold, I can carbonize the surfaces or by sufficiently long treatment in the retort 10 can carbonize the sheet metal quite through, in such cases preferably hardening by the heat used to carbonize.

I claim as my invention—

1. As an improved article of manufacture, 15 a freely-tumbling star composed of an angu-

lar piece of sheet-steel, dished, crimped and hardened, and externally presenting the radial angular edges substantially as herein specified.

2. In a tumbling-star, an angular piece of 20 sheet-steel dished, having its several points bent hookwise as indicated by A<sup>3</sup>, the whole star hardened, as herein specified.

In testimony that I claim the invention above set forth I affix my signature in presence of two witnesses.

GEO. D. BARTLETT.

Witnesses:

FLORA L. BARTLETT,  
FRED W. BARTLETT.